

## UNITED STATES PATENT OFFICE

2,551,644

METHOD OF PREPARING SYNTHETIC  
LUBRICANTS FROM ALPHA OLEFINS

Francis M. Seger, Pitman, William E. Garwood, Haddenfield, and Alexander N. Sachanen, Woodbury, N. J., assignors to Secony-Vacuum Oil Company, Incorporated, a corporation of New York

No Drawing. Application April 21, 1949,  
Serial No. 88,908

9 Claims. (Cl. 260—683.1)

1

This invention has to do with synthetic lubricants and, more particularly, has to do with polymerization of certain olefins to form a novel class of synthetic lubricants.

As disclosed in copending application Serial No. 761,716, filed July 17, 1947, by two of the present applicants, now abandoned in favor of application Serial No. 104,932, filed July 15, 1949, now Patent No. 2,500,166, it has been found that normal, alpha mono-olefins containing from six to about twelve carbon atoms per molecule polymerize, in the absence of a catalyst and under certain well-defined reaction conditions, to form synthetic lubricants. The lubricants so formed possess a highly desirable combination of properties: low pour point, high viscosity index and good stability. With regard to stability, however, these lubricants are characterized by the same degree of resistance to oxidation as the highly-refined Pennsylvania type lubricating oils. As is well recognized in the art, the latter oils are excellent lubricants in most respects but, under the rigorous conditions to which they are subjected in current internal combustion engines and the like, they do not possess sufficient resistance to oxidation. This has led to the development of numerous materials, "oxidation inhibitors" or "antioxidants," which are blended in the oils in minor amounts to inhibit oxidation. Yet, while these inhibitors are of considerable value in reducing the deleterious effects of oxidation upon Pennsylvania type lubricants and upon the aforesaid synthetic lubricants, they represent an added cost in the production of the oils.

It has now been found that the aforesaid normal, alpha mono-olefins polymerize, in the presence of a mercaptan or thiol, to form synthetic lubricants possessed of a substantially higher degree of oxidation stability as well as high viscosity index and low pour point. The invention comprises, therefore, the production of excellent synthetic lubricants by polymerization of a normal, alpha mono-olefin having from six to about twelve carbon atoms per molecule, at an elevated temperature from about 600° F. to about 750° F. in the presence of a minor amount, from about 0.001 to about 0.1 molar proportion (per molar proportion of olefin), of a thiol.

## REACTANTS

As indicated above, the mono-olefins of this invention include monomeric normal or straight-chain alpha, mono-olefins and contain from six to about twelve carbon atoms per molecule. Such mono-olefins are normally liquid at temperatures of the order of 20–25° C. Illustrative of such olefins are: hexane-1, octene-1, decene-1, and dodecene-1, and the like. Preferred of such olefins, however, are those having from eight to twelve carbon atoms per molecule, with decene-1

2

forming particularly outstanding synthetic lubricants. It will be clear from the foregoing examples that an alpha olefin may also be referred to as a 1-olefin.

Not only may the mono-olefins of the aforesaid character be used individually in this invention, but they may also be used in admixture with each other. In addition, olefin mixtures containing a substantial proportion of such mono-olefins may be used. Preferred of such mixtures are those containing a major proportion of a 1-olefin or of 1-olefins. Representative of such mixtures are those obtained by the cracking of paraffin waxes and other paraffin products, and those obtained from the Fischer-Tropsch and related processes. These hydrocarbon mixtures may contain, in addition to the 1-olefin or 1-olefins, such materials as: other olefins, paraffins, naphthenes and aromatics.

20 The mercaptan or thiol used herein may have an alkyl, aralkyl, alkenyl, aralkenyl, cycloalkyl, aryl, alkaryl, alkenylaryl, heterocyclic group etc. attached to the characterizing —SH group. Representative of such thiols or mercaptans are 25 the following: alkyl-methyl, ethyl, propyl, n-butyl, secondary butyl, isobutyl, hexyl, heptyl, octyl, dodecyl, etc.; aralkyl-benzyl, methyl benzyl, dimethyl benzyl and the like; alkenyl-vinyl, allyl, octadecenyl, etc.; aralkenyl-cinnamyl, styryl, 30 etc.; cycloalkyl-cyclopentyl, cyclohexyl, methyl cyclohexyl, methyl cyclopentyl, etc.; aryl-phenyl (thiophenol), naphthyl (thionaphthol), anthryl (thianthranol), etc.; alkaryl-tolyl, xylyl, methyl naphthyl, etc.; alkenylaryl-vinyl phenyl, allyl phenyl, etc.; heterocyclic-thiophenethiol, thi-anthrenethiol, benzthiophenethiol, pyridine thiol, etc. Thiophenethiol and its homologs, together with methods for their preparation are described in copending application Serial No. 40 721,454, filed January 10, 1947 now Patent No. 2,515,242.

Derivatives or substituted thiols may also be used herein, typical of which is mercapto ethanol. It will also be understood that polymercaptans or polythiols may be used. Illustrative of the latter is dithioglycol. The preferred thiols, however, are thiophenethiol, thiophenol, and n-butyl mercaptan.

## REACTION CONDITIONS

50 Polymerization of the aforesaid 1-olefins with the thiols is effected under critical conditions. Temperatures as low as about 300° F. and as high as the cracking temperatures of the lubricants formed, about 700° F., may be used. However, the temperature range of about 550° F. to about 650° F. is considered optimum in view of the unusually high degree of excellence of the lubricants formed under such conditions.

60 Polymerization is generally complete in from

one to twenty hours, preferably three to ten hours. It should be noted that reaction temperatures and times are interrelated, with the higher temperatures being used for the shorter reaction periods, and with the lower temperatures being used for the longer reaction periods.

The quantity of thiol or mercaptan used during the polymerization is, as indicated above, a relatively small quantity. This is a critical feature, for the quantity of thiol should not fall below about 0.001 molar proportion and preferably not exceed about 0.1 molar proportion, for each molar proportion of 1-olefin. When the quantity of thiol falls below the minimum indicated, little or no improvement in oxidation stability is realized. Similarly, when the maximum quantity of thiol is exceeded, the lubricant product generally contains an excessive quantity of sulfur, which restricts its use. Lubricants of the latter character, however, are particularly advantageous as blending stocks for mineral oils, such as Pennsylvania type oils, for they impart oxidation stability to the oils with which they are blended.

Pressures ranging from atmospheric to 1,000 pounds per square inch, most frequently about 300 pounds, characterize the polymerization. It is desirable to use sufficient pressure to maintain the olefins and thiols in liquid state.

It will be understood, of course, that the polymerization is aided by providing mixing of the olefins and thiols. This may be provided by using various agitating means which are well known in the art. At the polymerization or reaction conditions, the olefins and thiols are mutually soluble and homogeneity is readily attained.

Following the polymerization procedure, it is generally advisable to treat the reaction product to remove any unreacted thiol and any relatively low boiling sulfur-containing products. This may be accomplished by any of the conventional procedures for removing thiols or mercaptans from hydrocarbon mixtures. For example, aqueous alkali solutions may be used. So also may "solutizer solutions."

#### EXAMPLES

In order to illustrate the principles of this invention, the results of a series of typical, and non-limiting, polymerizations are set forth in tabular form in Table I below. These polymerizations were carried out in a rocking-type bomb (American Instrument Co.). An olefin and a thiol were charged to a bomb, the free space was swept with nitrogen, and the bomb was heated to the desired temperature for the

desired length of time. Thereafter, the bomb was cooled and discharged. It should be noted that the reaction times, recited as "Time, hours" in Table I, represent the time intervals during which the bomb was maintained at the desired temperature; and do not include the time intervals necessary to heat the bomb and its content to the desired temperature, and do not include the time intervals necessary to cool the bomb after heat to the bomb has been discontinued. Normally, about one and one-half hours are required to raise the temperature of the bomb from 70° F. to about 600° F.; similarly, several (about eight to sixteen) hours are required for the bomb to cool to 70° F. after being maintained at 600° F. for five hours.

The reaction or polymerization products discharged from the bomb were topped and filtered as indicated in the runs shown in Table I. To distinguish the synthetic lubricants from the crude reaction products and distillate fractions thereof, the refined oils are identified in Table I as "residual oils." The latter term identifies the oils from which unreacted materials and products of intermediate boiling range have been separated.

All of the tests and analyses to which the residual oils in Table I were subjected are well known standard tests. In this connection, it will be noted that the designation "N. N." refers to the neutralization number, which is a measure of the acidity of the oil. The abbreviation "K. V. at 210° F., cs." is used to identify the kinematic viscosity (of the residual oils) at 210° F., measured in centistokes.

By way of illustration, the procedure followed in run 8 (Table I) is provided in detail. Decene-1, 280 parts by weight or two molar proportions, and thiophenethiol, three parts by weight or 0.026 molar proportion, were charged to a stainless steel, rocking-type bomb. The bomb was pressured to approximately 1,600 pounds per square inch with nitrogen in order to check for leaks, pressure was released, and the system was closed. The bomb was then heated to 600° F. in approximately one and one-half hours, and maintained at 600-626° F. for ten hours (maximum pressure, 200 pounds per square inch). The reaction product, 281 parts by weight, was discharged from the bomb to a distillation flask and topped at a pressure of 8 mms. (Hg) to a maximum liquid temperature of 231° C. (448° F.). The residual oil, 86 parts by weight, was filtered through a thin coat of a diatomaceous earth filter aid, Super Filtrol, and the filtrate, 78 parts by weight was analyzed.

TABLE I

Reaction Conditions

| Run                                   | Olefinic Charge      | Parts by Weight | Moles | Mercaptan           | Parts by Weight | Moles | Temp., °F. | Time, Hrs.        | Max. Press., p. s. i. g. |
|---------------------------------------|----------------------|-----------------|-------|---------------------|-----------------|-------|------------|-------------------|--------------------------|
| POLYMERIZATION OF OLEFINS WITH THIOLS |                      |                 |       |                     |                 |       |            |                   |                          |
| 1                                     | Octene-1.....        | 336             | 3     | Thiophenethiol..... | 1               | 0.009 | 652        | 10 <sup>1/2</sup> | 700                      |
| 2                                     | Octene-1.....        | 336             | 3     | do.....             | 5               | 0.043 | 652        | 10                | 1,000                    |
| 3                                     | Octene-2.....        | 336             | 3     | do.....             | 1               | 0.009 | 650        | 10                | 750                      |
| 4                                     | Octene-2.....        | 366             | 3     | do.....             | 5               | 0.043 | 652        | 10                | 800                      |
| 5                                     | 2-Ethylhexene-1..... | 366             | 3     | do.....             | 1               | 0.009 | 645        | 10 <sup>1/2</sup> | 800                      |
| 6                                     | 2-Ethylhexene-1..... | 366             | 3     | do.....             | 5               | 0.043 | 652        | 10                | 850                      |
| 7                                     | Decene-1.....        | 420             | 3     | do.....             | 5               | 0.043 | 501        | 10                | 200                      |
| 8                                     | Decene-1.....        | 280             | 2     | do.....             | 3               | 0.026 | 610        | 10                | 200                      |
| 9                                     | Decene-1.....        | 420             | 3     | do.....             | 5               | 0.043 | 635        | 10                | 150                      |
| 10                                    | Decene-1.....        | 420             | 3     | do.....             | 5               | 0.043 | 700        | 3                 | 1,250                    |
| 11                                    | Decene-1.....        | 420             | 3     | do.....             | 5               | 0.043 | 750        | 3                 | 2,300                    |

TABLE I—Continued

| Run                                   | Olefinic Charge | After Treatment     | Residual Oil    |                                 |                      |                      |       |                 |       |                  |                  |            |
|---------------------------------------|-----------------|---------------------|-----------------|---------------------------------|----------------------|----------------------|-------|-----------------|-------|------------------|------------------|------------|
|                                       |                 |                     | Parts by Weight | Wt. Per Cent Yield <sup>1</sup> | K. V. @ 100° F., cs. | K. V. @ 210° F., cs. | V. I. | Pour Point, °F. | N. N. | Specific Gravity | Color (Lovibond) | Per Cent S |
| POLYMERIZATION OF OLEFINS WITH THIOLS |                 |                     |                 |                                 |                      |                      |       |                 |       |                  |                  |            |
| 1                                     | Octene-1        | Topped <sup>2</sup> | 33              | 9.8                             | 11.54                | 2.80                 | 93    | <-30            | 0.1   | —                | 3                | 2.81       |
| 2                                     | Octene-1        | do <sup>2</sup>     | 32              | 9.4                             | 11.61                | 2.74                 | 77.7  | <-30            | 0.1   | —                | —                | 1.53       |
| 3                                     | Octene-2        | do <sup>2</sup>     | 21              | 6.2                             | 13.26                | 3.02                 | 88    | <-30            | 0.2   | —                | —                | —          |
| 4                                     | Octene-2        | do <sup>2</sup>     | 26              | 7.6                             | 13.79                | 3.01                 | 71.5  | <-30            | 0.1   | —                | 7—               | 3.98       |
| 5                                     | 2-Ethylhexene-1 | do <sup>2</sup>     | 8               | 2.4                             | Insufficient Sample  |                      |       | —               | —     | —                | —                | —          |
| 6                                     | 2-Ethylhexene-1 | do <sup>2</sup>     | 13              | 3.8                             | 16.99                | 3.22                 | 36.5  | <-30            | —     | —                | —                | —          |
| 7                                     | Decene-1        | Topped <sup>3</sup> | 12              | 2.8                             | 14.23                | 3.35                 | 122   | <-30            | —     | —                | 11.64            | —          |
| 8                                     | Decene-1        | do <sup>3</sup>     | 86              | 30.4                            | 6.27                 | 2.01                 | 122.6 | -30             | 0.1   | 0.8296           | 33               | 2.48       |
| 9                                     | Decene-1        | do <sup>3</sup>     | 217             | 51                              | 7.55                 | 2.24                 | 116.5 | -20             | Nil   | 0.8222           | 0.8              | 0.85       |
| 10                                    | Decene-1        | do <sup>3</sup>     | 59              | 13.9                            | 15.78                | 3.56                 | 121.4 | -15             | 0.2   | 0.8428           | 1                | 1.10       |
| 11                                    | Decene-1        | do <sup>3</sup>     | 31              | 7.3                             | 30.76                | 5.14                 | 105.5 | -30             | 0.1   | 0.8729           | 160              | 0.83       |

<sup>1</sup> Overall yield, based on original charges.<sup>2</sup> First topped at atmospheric pressure to a maximum liquid temperature of 200° C., then topped at pressure of 1-4 mm. to a maximum liquid temperature of 140-200° C. Residue filtered through thin coat of Super Filtral.<sup>3</sup> Topped at pressure of 1-8 mm. to a maximum liquid temperature of 190-231° C. Residue filtered through coat of Super Filtral.

From the data in Table I, it will be seen in runs 1-6, that a substantially larger yield of synthetic oil is obtained from octene-1 (a normal, alpha mono-olefin) than from either octene-2 or 2-ethylhexene-1. The octene-2 used in runs 3 and 4 (as obtained from a commercial source) contained an appreciable quantity of octene-1 and, therefore, the actual difference between the two octenes, -1 and -2, is much greater than shown here. There is also a significant difference in viscosity indices of the residual oils, with the oils obtained from octene-1 being markedly superior. It is also noteworthy that as the quantity of thiophenethiol is increased, the viscosity index of the residual oil is decreased.

Runs 7-11 show the effect of temperature and time upon the polymerization of decene-1 in

Dry air is passed through the sample of oil at a rate of ten liters per hour. The test tube is heated at 260° F. for forty hours in an aluminum block bath. The results reported at the end of the test are: neutralization number (N. N.); per cent viscosity increase at 210° F.; sludge and lacquer; lead weight loss (in milligrams); and appearance of copper. The oil is compared with a reference oil of similar viscosity and is rated on the basis of viscosity increase, N. N. increase, sludge and lead weight loss. A maximum of three demerits is assigned to each factor rated. The sum of the demerits for an oil is called the stability number and ranges from zero to twelve. The reference mineral oils, solvent-refined Pennsylvania oils, have a stability number of six to seven.

TABLE II  
Catalytic oxidation test

| Oil                                                                   | N. N. (SV) | K. V. @ 210° F., cs. | Per Cent Vis. Inc. | Sludge, Tube | Copper Coil | Pb Loss, Mg | Stability Number |
|-----------------------------------------------------------------------|------------|----------------------|--------------------|--------------|-------------|-------------|------------------|
| SAE 10W Pennsylvania Mineral Oil <sup>1</sup>                         | 16         | 12.91                | 125                | Nil          | —           | 235         | 6 or 7           |
| PRODUCTS FROM REACTION OF MERCAPTANS DURING POLYMERIZATION OF OLEFINS |            |                      |                    |              |             |             |                  |
| Run 8                                                                 | 0.5        | 2.09                 | 3.9                | Nil          | Brown       | 26.5        | 0                |
| Run 9                                                                 | 1.7        | 2.44                 | 8.9                | do           | Gray Stain  | 44.3        | 0                |

<sup>1</sup> Averaged values.

the presence of thiophenethiol. The results reveal that time-temperature conditions of ten hours at about 600° F. to three hours at 700° F. is most advantageous. It is apparent that at temperatures of about 500° F., yield of oil is low and sulfur content of the oil is relatively high. Similarly, with a temperature of 750° F. and a reaction time of three hours, viscosity index is substantially lower than at 700° F. for the same time period.

That the residual oils of this invention have excellent stability is shown by results of a catalytic oxidation test, the results being shown below in Table II. This oxidation test reveals the stability of oils toward catalytic oxidation.

The test oil, 25 ccs., is placed in a 200 x 25 mm. test tube with 15.6 square inches of sand-blasted iron wire, 0.78 square inch of polished copper wire, 0.87 square inch of polished aluminum wire, and 0.167 square inch of polished lead plate.

The test data set forth in Table II clearly indicate the high degree of stability which characterizes the oils contemplated herein; and demonstrate their superiority in this regard over a Pennsylvania type mineral oil and a lubricant obtained by thermally polymerizing a normal, alpha mono-olefin, decene-1, in the absence of a thiol.

As will be evident from the data presented above in Tables I and II, the polymerization products of this invention are highly desirable lubricants per se. They are also of considerable value as blending agents for other lubricating oils. In view of the inherent stability of the synthetic oils, they impart stability to the oils with which they are blended. So also, they impart desirable viscosity index (V. I.) and pour point characteristics to the oils in combination therewith, for, as indicated above, they have advantageous viscosity index and pour point properties. In short, the

synthetic oils find utility in "upgrading" other lubricants. Typical oils with which the synthetic oils may be blended are mineral oils such as are normally used in internal combustion and turbine engines. When so blended, the synthetic oils may comprise the major proportion of the final blended oil, or may even comprise a minor proportion thereof. For example, although used only in the amounts of the order of one to ten per cent, the synthetic oils improve the stability of mineral oils, such as SAE 10 and 20 Pennsylvania type oils.

One or more of the individual properties of the synthetic lubricants of this invention may be further improved by incorporating therewith a small, but effective amount, of an addition agent such as an antioxidant, a detergent, an extreme pressure agent, a foam suppressor, a viscosity index (V. I.) improver, etc. Antioxidants which may be used are well-known in the art, and are generally characterized by phosphorus, sulfur, nitrogen, etc. content; representative of such materials is a phosphorus- and sulfur-containing reaction product of pinene and  $\text{P}_2\text{S}_5$ . Typical detergents which may be so used are metal salts of alkyl-substituted aromatic sulfonic or carboxylic acids, as illustrated by diwax benzene barium sulfonate and barium phenate, barium salt of a wax-substituted phenol carboxylic acid. Extreme pressure agents are well known; illustrating such materials are numerous chlorine and/or sulfur containing compositions, one such material being a chlornaphtha xanthate. Silicones, such as dimethyl silicone, may be used to illustrate foam suppressing compositions. Viscosity index improving agents which may be used are typified by polypropylenes, polyisobutylenes, polyacrylate esters, and the like.

Contemplated also as within the scope of this invention is a method of lubricating relatively moving surfaces by maintaining therebetween a film consisting of any of the aforesaid oils.

We claim:

1. A method of preparation of a viscous oil characterized by low pour point, high viscosity index and high oxidation stability, which comprises: non-catalytically heating a hydrocarbon charge consisting essentially of a normal, alpha mono-olefin having from six to about twelve carbon atoms per molecule in the presence of a thiol, the molar ratio of said thiol to said olefin being

from about 0.001 to about 0.1, at a temperature between about 300° F. and about 700° F.

2. The method of claim 1 wherein the temperature is maintained between about 550° F. and about 650° F. for a period of time between about ten hours and about three hours, respectively.

3. The method of claim 1 wherein said molar ratio is from about 0.005 to about 0.05.

4. The method of claim 1 wherein the mono-olefin is a monomer having from about eight to about twelve carbon atoms per molecule.

5. The method of claim 1 wherein the thiol is an alkyl thiol.

6. The method of claim 1 wherein the thiol is an aryl thiol.

7. The method of claim 1 wherein the thiol is a heterocyclic thiol.

8. The method of preparation of a viscous oil characterized by low pour point, high viscosity index and high oxidation stability, which comprises: non-catalytically heating a charge consisting essentially of one molar proportion of n-decene-1 and about 0.015 molar proportion of thiophenethiol, at about 635° F. for about ten hours.

9. The method of preparation of a viscous oil characterized by low pour point, high viscosity index and high oxidation stability, which comprises: non-catalytically heating a charge consisting essentially of one molar proportion of n-octene-1 and about 0.003 molar proportion of thiophenethiol, at about 650° F. for about ten hours.

FRANCIS M. SEGER.  
WILLIAM E. GARWOOD.  
ALEXANDER N. SACHANEN.

#### REFERENCES CITED

The following references are of record in the file of this patent:

#### UNITED STATES PATENTS

| Number    | Name               | Date          |
|-----------|--------------------|---------------|
| 2,258,806 | Pier et al. -----  | Oct. 14, 1941 |
| 2,382,700 | Eby -----          | Aug. 14, 1945 |
| 2,486,441 | Segar et al. ----- | Nov. 1, 1949  |

#### OTHER REFERENCES

Egloff: "The Reactions of Pure Hydrocarbons" (Reinhold Publ. Corp., 1937), pages 362-363.